

Sept. 2, 1930.

C. H. BRASELTON

1,774,698

VACUUM TUBE FILAMENT CONNECTION AND METHOD OF CONNECTING

Filed Jan. 25, 1928

Fig. 1.



Fig. 2.



INVENTOR

*Chester H. Braselton*

## UNITED STATES PATENT OFFICE

CHESTER H. BRASELTON, OF NEW YORK, N. Y., ASSIGNOR TO ARCTURUS RADIO TUBE COMPANY, OF NEWARK, NEW JERSEY, A CORPORATION OF DELAWARE

## VACUUM-TUBE-FILAMENT CONNECTION AND METHOD OF CONNECTING

Application filed January 25, 1928. Serial No. 249,261.

This invention relates to vacuum tubes and more particularly to a method of connecting the ends of the filaments commonly used in such tubes.

One of the objects of the invention is to provide a connection between a filament and the support therefor which will not be injuriously affected by the heat of the filament.

Another object of the invention is to provide a method of connecting the ends of filaments to supports whereby the connection is protected from the excessive heat of the filament.

Another object of the invention is to provide means to conduct heat rapidly away from the ends of the filament.

Another object of the invention is to provide a method of reinforcing the ends of a filament adjacent the supports therefor.

Another object of the invention is to provide a means to increase the conductivity of the ends of the filament to reduce the heating effect of the current therein.

Other objects of the invention will be apparent as the description proceeds.

One embodiment of the invention has been illustrated in the accompanying drawing in which:

Fig. 1 is an elevation of a vacuum tube embodying my invention; and

Fig. 2 is an enlarged view of the filament showing the means to connect it at each end of the support.

Referring now more particularly to the drawing, the invention has been shown in connection with a vacuum tube of the heater type such as is shown and described in the copending application of Walter L. Krahl "vacuum tube construction and circuit therefor" S. N. 156,947 filed December 24, 1926.

This vacuum tube comprises an envelope 10 mounted on the usual base (not shown) which carries the necessary terminals for connecting the vacuum tube to the circuit 45 of the radio set. A press 11 is provided within the envelope into which the various supports for the elements are sealed. A tubular plate 12 is supported on conductor rods (not shown) and a cylindrical grid 13 is 50 mounted inside of the plate 12 in a manner

well known in the art. A tubular electron-emitting cathode 14 is also mounted within the plate and grid and a carbon filament 15 is positioned within the cathode and forms the heater therefor. This filament 15 is supported on its lower end upon the conductor 16 while its upper end is connected by means of a spring wire 17 to the upper end of a support 18 which also forms the support for the upper end of the cathode 14.

Considerable difficulty has been experienced in connecting the ends of the filament 15 to their supports. In some instances metal tabs have been used which have been attached to the filament and in turn welded to the supports, but some objection has been found to this method of attaching the ends, inasmuch as it is difficult to attach the tabs to the carbon of the filament without damaging the ends of the filament and causing possible failure after a short use of the tube. In the present invention I have found that by copper plating the ends of the carbon they may be welded directly to a support, which results in a simpler and more secure connection. This is true especially of the lower end of the filament which is welded to a nickel support 16. The upper end of the filament, however, is preferably attached to the spring 17 which may be made of phosphor bronze, for instance, or any other spring wire which cannot readily be welded to copper, and it is desirable, therefore, in securing the upper end of the filament, to nickel plate the end after the same has been copper plated and then weld the nickel plated end directly to the spring wire.

With the filament connected as indicated at its lower and upper ends there is some danger of the plating fusing, due to the high heat of the filament, which fusing may result in the evolution of gases or a general weakening of the connection, either of which might be detrimental to the operation of the tube. I have therefore found that if the juncture of the carbon with the plating on the filament is covered with a metallic paste, the paste not only acts as a reinforcing agent to strengthen the ends of the filament, and provides a means to rapidly con-

duct heat away from the ends of the filament as well as to protect the ends from the radiant heat of the filament and cathode which prevents any danger of the fusing of the plating thereon, but also increases the conductivity of the ends and lowers the temperature thereof which would otherwise be high due to the current flowing therethrough.

The construction is illustrated in Fig. 2 in 10 which the filament 15 is plated with copper 19 at both ends and has a further plating of nickel 20 at its upper end. The metallic paste 21 is shown surrounding the filament at the point where the plating begins.

15 Such a metallic paste is well known in the art and may consist of Dixon's graphite, caramel, gum arabic, cryolite, boracic acid, and silver nitrate. The paste is spread in a plastic state on the filament after the ends 20 have plated and then allowed to dry which takes approximately one half hour, or, it may dry in a shorter time if the temperature is increased.

25 This means of connecting the upper and lower end of the filament, as is evident from the above description, is simple and very effective, and while I have shown and described one embodiment of the invention, it is evident that variations may be made in the manner of making the connection and in the type 30 of metal and composition of the paste used without departing from the spirit of the invention, and I do not, therefore, desire to limit myself to the specific means and method 35 shown and described, but to interpret the invention broadly within the scope of the appended claims.

What I claim is:

40 1. The method of attaching a carbon filament to a support which comprises plating the end of the filament, applying a heat conducting paste to the plated end, and welding said end to a support.

45 2. The method of attaching a carbon filament to a support which comprises plating the end of the filament, applying a reinforcing paste to the plated end and welding the plated end to a support.

50 3. The method of connecting a carbon filament to a support which comprises plating the end of the filament, covering a portion of the plated end with a metallic heat conducting paste and welding the end of the filament to a support.

55 4. The method of welding a carbon filament to a support which comprises copper plating the end of the filament, covering a portion of the said end with heat conducting paste, and welding said end to a support.

60 5. The method of attaching a carbon filament to a spring support which comprises copper plating the end of the filament, nickel plating said end over the copper plate, covering a portion of said end with a coating of

heat conducting paste, and welding said end to a spring support.

6. The method of attaching a carbon filament to a spring support which comprises copper plating the end of said filament, nickel plating said end over the copper plate, covering a portion of said end with a coating of metallic paste, whereby said end is reinforced and welding said end to the spring support.

7. In a vacuum tube a carbon filament, a metallic plating on the end of said filament and a coating of heat conducting material on the filament at the juncture of the filament and plating.

8. In a vacuum tube a carbon filament, a metallic plating on the end of said filament and a coating of electrical conducting material on said filament at the juncture of the filament and plating.

9. In a vacuum tube a carbon filament, a metallic plating on the end of said filament, and a reinforcing material at the juncture of the filament and the plating to protect the plating from the excessive heat of the filament.

10. In a vacuum tube, a filament of high resistance material, a metallic plating on the end of said filament and a coating of metallic paste over the juncture of said filament and plating to protect said plating from the heat of said filament.

In testimony whereof, I affix my signature.

CHESTER H. BRASELTON.

100

105

110

115

120

125

130